

## UNITED STATES PATENT OFFICE

MICHAEL GEORGE CORSON, OF JACKSON HEIGHTS, NEW YORK

## PROCESS OF REFINING (DEGASIFYING AND DEOXIDIZING) OF COPPER

No Drawing. Application filed April 26, 1927, Serial No. 186,821. Renewed November 12, 1929.

The present day practice of refining copper and particularly of remelting either cathode or native copper embraces among its various aims those of removing sulfur, which is done by a process of oxidation and of removing the oxygen, which is done by poling.

The first named impurity is rarely present in amounts larger than 0.050% and frequently passes into practically pure copper (cathodes) by absorption from the gases resulting from the combustion of various low grade fuels used in melting the same, sulfur usually being an unavoidable component of such gases. While the theoretical amount of oxygen required for the "oxidation" of this sulfur ought not to be larger than the amount of sulfur itself, the practical amount of oxygen permitted to combine with copper in the oxidation process runs, however, beyond 0.5% and sometimes up to 1.0% of the total weight of the metal. In other words, an excess of oxygen amounting to 1000-2000% is considered necessary for the complete removal of sulfur.

25 This large amount of oxygen calls in its turn for a prolonged period of poling and for a considerable consumption of wooden poles. Again, the operation of poling has to be closely watched, since the overpolished material will 30 contain absorbed hydrogen and the ingots cast of it will be gassed.

I have found that neither the excessive oxidation, nor the prolonged poling are really necessary. I have found that the process of 35 "oxidation" pertains only to copper and not to sulfur, since there is always enough oxygen in the copper during its sojourn in the furnace to take care of the sulfur by forming  $SO_2$  gas. The "oxidation" is only a secondary 40 phenomenon to the blowing away of the low pressure layer of sulfur dioxide gas covering the surface of the molten metal. This blowing away of sulfur dioxide destroys the equilibrium between the sulfur dioxide on the one hand and sulfur plus oxygen on the other, as dissolved in copper, and as a consequence a 45 continuous evaporation of sulfur dioxide takes place.

I have discovered that the removal of sulfur, i. e., sulfur dioxide, will take place with-

out over-oxidizing copper if the molten metal is kept under vacuum. With the total gas pressure over the molten copper maintained at say 1-5" of mercury, a rapid and practically complete removal of sulfur dioxide 55 takes place and the molten metal can be made to contain not more than 0.10% oxygen.

My invention also includes the removal of the oxygen from the molten copper. While poling may be retained for the elimination of 60 the bulk of oxygen, it cannot result in a sound metal, unless about 0.04% of oxygen are allowed to remain in the metal. This amount of oxygen produces about 9% by volume of a copper-copper-monoxide eutectic and the latter causes a large number of troubles in various industrial applications of copper.

All other methods of a complete deoxidation of copper proposed and used until the present, consist in the introduction of some 70 reducing agent, which for the sake of efficient use must be soluble in copper. The amount of this reducing substance cannot be strictly calculated and has to be introduced in a considerable excess. This results either in 75 the formation of a solid solution (in case of phosphorus, silicon and manganese) or of a secondary constituent—a compound of copper with the reducing agent (in the case of magnesium, calcium, cerium). In the first 80 case the electric conductivity is impaired, in the second the metal is likely to be dirty and to cause troubles in its future uses.

Other reducing agents, for instance boron suboxide and calcium carbide have been suggested and actually used. These substances remain, however, solid at the melting point of copper and float upon the latter's surface, whence their reducing action may not be efficient and reliable.

I have found that calcium carbide may 85 form a cheap and highly efficient reducing agent provided it is present in a liquid form. For this purpose I dissolve calcium carbide in some molten fluoride or a mixture of fluorides. Among these sodium fluoride, calcium fluoride, aluminum-sodium fluoride (cryolite) represent good solvents for calcium carbide. A mixture of fluorides with chlorides 90 may also be used quite efficiently.

In general, my process of refining copper may be presented as follows:

Cathode or native copper is continuously melted in the usual type of reverberatory furnace and amounts of the molten metal are withdrawn periodically and placed in an auxiliary furnace of some kind, which is so arranged as to make it possible to close it reasonably airtight so enabling a strong vacuum pump to produce a vacuum with a remaining pressure of 1-5''. In a few minutes the total amount of sulfur is eliminated as sulfur dioxide. Next the molten metal is covered with a roughly powdered mixture of fluorides and calcium carbide, though it is also possible to introduce this mixture in a liquefied form. A violent reaction starts immediately and after a few minutes the layer of the reducing mixture becomes quiet which indicates the end of reduction (deoxidation); the metal is immediately ready for pouring, and no contamination of any kind results.

This process of deoxidizing with the aid of a liquid layer of a mixture of fluorides and calcium carbide is not limited to use in conjunction with the removal of sulfur dioxide by the application of a vacuum. It can be as well applied to the molten oxidized copper resulting from the process of removing sulfur by "oxidation" as is usually done in the refineries. It can also be used as a supplementary method to completely deoxidize copper, which has been previously partly deoxidized by poling.

It is to be understood that the invention is not limited to the treatment of copper metal but may also be applied to the manufacture of copper alloys. The molten copper or copper alloy is covered with a layer of a mixture of fluorides and calcium carbide for example two lbs. of sodium fluoride and one-half lb. of calcium carbide to 100 lbs. of copper. The carbide immediately frees the copper from oxygen and other metals added to copper will not, therefore, become oxidized and no film of any oxide may be found in alloys manufactured in this way.

Claims:

1. A process of purifying copper which comprises forming a bath of metal, oxidizing any sulfur present to sulfur dioxide, and then lowering the pressure upon the surface of the bath to a point substantially below atmospheric, and maintaining such condition until the sulfur dioxide has been removed.

2. A process of purifying copper which comprises forming a bath of metal, oxidizing any sulfur present to sulfur dioxide, then lowering the pressure upon the surface of the bath to a point substantially below atmospheric and maintaining such condition until the sulfur dioxide has been removed, and then treating with a mixture of calcium carbide and fluorides capable of dissolving the car-

bide at the temperature of the molten metal to deoxidize the same.

3. A process of deoxidizing copper which comprises treating the oxygen-containing metal while molten with a mixture of calcium carbide and fluorides capable of dissolving the carbide at the temperature of the molten metal. 70

4. A process of deoxidizing copper which comprises treating the oxygen-containing metal while molten with a mixture comprising calcium carbide and sodium fluoride. 75

5. A process of deoxidizing copper which comprises placing a mixture of calcium carbide and fluorides upon the surface of a bath of copper, the fluorides being so chosen and present in such amount as to insure the dissolution of the calcium carbide in the fluorides under the influence of the heat of the bath, and maintaining the bath fluid until 85 the copper has become substantially deoxidized.

6. A process of deoxidizing a copper-containing bath which comprises forming a layer of molten fluorides upon the bath, dissolving calcium carbide therein, and maintaining the bath fluid until it has become substantially deoxidized. 90

7. A process of deoxidizing copper which comprises treating the oxygen-containing metal while molten with a mixture comprising calcium carbide and cryolite. 95

Signed at 8108 Polk Ave. Jackson Heights in the county of Queens and State of New York this twenty-third day of April A. D. 1927. 100

MICHAEL GEORGE CORSON.

105

110

115

120

125

130